

## UNITED STATES PATENT OFFICE

2,381,219

## ALUMINUM ALLOY

Ira M. Le Baron, Arnold, Pa., assignor to Aluminum Company of America, Pittsburgh, Pa., a corporation of Pennsylvania

No Drawing. Application October 12, 1942,  
Serial No. 461,721

6 Claims. (CL. 75—139)

This invention relates to aluminum base alloys and more particularly to aluminum base alloys containing substantial amounts of copper and small amounts of other specific alloying elements for improving the tensile properties of the alloy in the heat treated and precipitation hardened condition.

Aluminum-copper alloys, particularly those aluminum base alloys containing between 1 and 12 per cent copper, have found wide application in industry and have been used in large quantities. Although these alloys in either the as-cast or as-wrought condition exhibit satisfactory tensile properties and resistance to corrosion for many purposes, their tensile strength and hardness may be considerably increased by solution heat treatment and subsequent aging. There are, however, certain uses for which these alloys are employed, which require exceptionally high tensile properties together with good resistance to corrosion and good working and machining characteristics. Furthermore, these high properties whether in the cast or wrought alloy must remain relatively stable over long periods of time under all operating conditions. A notable example of the uses requiring alloys having the foregoing properties is found in the fabrication of aircraft. The high minimum requirements for the aluminum-copper alloys in the aircraft industry are generally easily met and the properties remain within relatively narrow limits indefinitely so that good performance of these light alloys is obtained; however, constant effort is being made to improve them in order that the current minimum requirements will be greatly exceeded.

It is an object of the present invention to provide a heat treatable aluminum base alloy containing appreciable amounts of copper, having high tensile properties and good resistance to corrosion. Another object of the present invention is to provide aluminum base alloys containing appreciable amounts of copper, which have good tensile properties and resistance to corrosion and which are greatly improved in tensile properties by heat treating and aging. Still another object of my invention is to provide aluminum base alloys containing appreciable amounts of copper, which possess good working and machining characteristics together with high tensile properties and good resistance to corrosion.

The term aluminum base alloy as used throughout the specification and appended claims refers to an alloy containing at least 70 per cent metallic aluminum by weight. The term aluminum-cop-

per alloy refers to an aluminum base alloy containing copper as the predominant added alloying element. The terms heat treatment and solution heat treatment as used herein signify a treatment wherein an alloy is heated to a temperature below the fusion point of the lowest melting eutectic of the alloy for a time sufficiently long to dissolve a substantial portion of the soluble alloying constituents. Artificial aging is a treatment given to precipitation hardening alloys, wherein the alloy is heated to a temperature somewhat above room temperature but below the heat treating temperature to precipitate the alloying ingredients present in the aluminum in a supersaturated condition, a condition produced by rapidly cooling the alloy from the solution heat treating temperature. The term tensile properties includes tensile and yield strength, elongation and hardness of the alloy.

The present invention is predicated on the discovery that the tensile properties and resistance to corrosion of solution heat treated and artificially aged magnesium-free aluminum base alloys containing copper are greatly improved by the addition to those alloys of about 0.01 to 2.0 per cent of lithium and at least one of the elements selected from the group, which for convenience may be called the cadmium group, consisting of cadmium, mercury, silver, tin, indium and zinc, these elements being present in the proportion of about 0.01 to 1.5 per cent each of cadmium, mercury, silver, tin, indium, and about 0.01 to 0.5 per cent of zinc, the total of these elements not exceeding about 1.5 per cent. The combination of lithium and one or more of the elements from the above group in the aluminum-copper alloys has the surprising effect of improving the tensile properties and resistance to corrosion to an extent much greater than the aggregative effect of the same elements present separately in the alloys. Lithium is not known to have any pronounced beneficial effect on the tensile properties of the alloy when not in combination with the elements of this group and it is sometimes even detrimental to the tensile properties; however, lithium with one or more elements from the cadmium group forms a combination which exerts an unexpected and profound influence on the properties of aluminum-copper alloys, and furthermore, to achieve the objects of the present invention lithium must be present in all combinations of elements from the foregoing group. Lithium should be present in the alloy in amounts not less than 0.01 per cent to consistently obtain any substantial improvement in properties, and

it need not be present in amounts greater than about 2.0 per cent, since in amounts over about 2.0 per cent lithium has no noticeable improvement on the properties of the alloy. The preferred range for lithium in the aluminum-copper alloys is between about 0.5 and 1.5 per cent.

Of the elements of the above cadmium group, cadmium is preferred because in addition to the beneficial effect of lithium-cadmium combination on the tensile properties of the alloys, cadmium is easily handled during production of the alloy and it does not have any particular detrimental effects on the alloy if the maximum limit is exceeded. Cadmium may be present in the alloy in amounts from 0.01 to 1.5 per cent but the most pronounced increase in tensile properties occurs when it is present in amounts between 0.02 and 0.5 per cent, and above about 1.5 per cent there is practically no increase in properties.

The combinations of lithium with tin, mercury, indium and silver also greatly improve the tensile properties of aluminum-copper alloys, but the influence of these combinations is not as pronounced as that of lithium and cadmium. The percentages of tin, mercury, indium and silver which should be added to the alloy with lithium are about the same as the percentages of cadmium, i. e., between 0.01 and 1.5 per cent and a preferred range between 0.02 and 0.1 per cent.

Zinc in combination with lithium has a beneficial influence on the tensile properties of aluminum-copper alloys, but as the amount of zinc increases the alloy becomes increasingly brittle until above about 0.5 per cent the alloy is so brittle that it is unsatisfactory for most uses. It is preferable to keep the zinc within a range from 0.01 to 0.05 per cent. The combination of lithium-cadmium-zinc will produce slightly better properties in the alloy than lithium and cadmium alone, but it is preferable to keep a low zinc content, such as between 0.01 and 0.05 per cent, and the combined amount of the cadmium and zinc should not exceed 1.5 per cent. While other combinations containing more than one metal from the cadmium group will produce substantial increases in tensile properties, it has been found that combinations using only one metal from the group usually have the greatest influence on the tensile properties. The lithium-cadmium-zinc combination is the only exception to this. When more than one metal from the group is employed in the combination the total amount of these metals should not exceed about 1.5 per cent.

In the combination of lithium and one or more of the metals from the cadmium group, no exact ratio of the metals to one another is required; however, the greatest improvement in tensile properties of the alloy without a substantial diminution of other desirable properties is obtained when the elements are present in the amounts falling within the preferred ranges given.

The elements of the group which form combinations with lithium and improve the properties of aluminum-copper alloys are also a natural group in which are elements possessing a number of similar chemical and physical properties, as for example, density, melting point, strength and affinity for oxygen. This is shown in the periodic system of the elements given in a table on page 5 in "The Principles of Physical Metallurgy," by Doan and Mahla, and explained on pages 4 and 6. Here all the metals in my group, except silver, are found in the "low melting heavy metals"

group. Silver, however, which is found adjacent to this group is characterized by many of the properties common to the metals of this group. From the effect displayed by the elements of the cadmium group on the aluminum-copper alloys and from the disclosure in Doan and Mahla, these elements must necessarily be considered as a group. Lithium which falls in the "light metals" group of this periodic system is definitely different in many of its physical and chemical properties from the elements in the low melting heavy metals group, and therefore cannot be considered in the class with the elements in that group.

The alloys to which the addition of lithium and one or more of the elements of the aforementioned group is particularly beneficial are those containing 1 to 12 per cent copper, not more than 1 per cent each of silicon and iron present as impurities, and with or without a total of 0.01 to 1.5 per cent of one or more of the hardening elements manganese, chromium, titanium, molybdenum, tungsten, vanadium, zirconium, nickel, cobalt, beryllium and boron within the following proportions for each of said elements: manganese, 0.05 to 1.5 per cent; chromium, 0.05 to 1 per cent; titanium, 0.03 to 0.5 per cent; molybdenum, 0.05 to 1 per cent; tungsten, 0.05 to 1 per cent; vanadium, 0.01 to 1 per cent; zirconium, 0.05 to 0.5 per cent; nickel 0.05 to 1 per cent; cobalt, 0.05 to 1 per cent; beryllium, 0.01 to 0.5 per cent; and boron, 0.01 to 0.5 per cent. The foregoing hardening elements constitute a group of substances all but the last two of which are in the "high melting heavy metals" group of the table in the book by Doan and Mahla previously referred to, and which, for the purposes of my invention, are alike in respect to their hardening effect upon the alloys of aluminum-copper-lithium and one or more metals from the cadmium group. Although beryllium and boron are not found in the high melting heavy metals group of this table, they have high melting points together with a number of characteristics similar to the metals in the high melting heavy metals group. All the above named elements serve to enhance particular properties of the alloy without substantially altering its fundamental characteristics. The preferred range for copper in these alloys is between 3 and 5 per cent.

The term magnesium-free alloys as herein employed refers to those alloys which have less than 0.01 per cent magnesium present as an impurity. Since magnesium has a definite detrimental effect on the tensile properties of my alloys, it is desirable in commercial practice to keep this impurity below a maximum of 0.005 per cent.

The solution and aging treatments for aluminum-copper alloys containing lithium and one or more metals from the cadmium group are not materially different from the conventional treatments given to aluminum-copper alloys, i. e., a solution treatment wherein the alloy is heated to a temperature sufficiently high and for a period of time sufficiently long to dissolve the soluble constituents. This heat treatment is conventionally carried out for aluminum-copper alloys at a temperature between 850-1000° F. for a period of time between 15 minutes and 8 hours. The alloy is then quenched and artificially aged. In the aging treatment the quenched alloy is held at a temperature between 250 and 400° F. for 4 to 20 hours. No special conditions or equipment are required to heat treat and age my alloys.

The improvement in aluminum-copper alloys

in the heat treated and aged condition by the addition of lithium and one or more metals from the cadmium group occurs in either the cast or wrought alloys and in addition to the high tensile properties and resistance to corrosion, these alloys possess good machining and working characteristics.

The effect of the combination of lithium and an element selected from the cadmium group on the tensile properties of aluminum-copper alloys may be illustrated from the following observations. An aluminum base alloy nominally containing 4.5 per cent copper, 0.8 per cent manganese, 0.25 per cent silicon and 0.15 per cent iron was melted and divided into three portions, one portion being used as a standard of comparison, and lithium and cadmium being added to one of the remaining portions, and lithium, cadmium and silver being added to the other remaining portion. The amounts of lithium, cadmium and silver in these portions are indicated in the table below. The ingots from each portion were poured under similar conditions and then rolled into sheet about  $\frac{1}{8}$  inch in thickness. Six standard test specimens were machined from each sheet and all were heat treated at 980° F. for 15 minutes, quenched in cold water and then artificially aged 12 hours at 320° F. The tensile properties of the alloys from each portion as shown by the average results from tests made on the specimens are listed in the following table:

| Alloy  | Per cent of Li in alloy | Per cent of Cd in alloy | Per cent of Ag in alloy | Tensile strength | Yield strength | Percent elongation |
|--------|-------------------------|-------------------------|-------------------------|------------------|----------------|--------------------|
| 1..... | None                    | None                    | None                    | 57,000           | 35,000         | 18.0               |
| 2..... | 1.0                     | 0.15                    | None                    | 82,195           | 75,900         | 7.8                |
| 3..... | 1.0                     | 0.15                    | 0.15                    | 80,650           | 74,500         | 7.5                |

The large improvement in the tensile properties of aluminum-copper alloys by the addition of lithium and one or more of the elements from the cadmium group is found only in the heat treated and aged alloys, and these heat treated and aged properties can be varied somewhat by selecting different heat treating and aging temperatures. From the results shown in the table of the tests made on the specimens from all three portions, the beneficial effect of lithium-cadmium and lithium-cadmium-silver combinations on the tensile properties of heat treated and artificially aged aluminum-copper alloys is apparent.

The claims wherein the phrase "the balance substantially all aluminum" is employed include the elements, particularly the hardening elements, which are frequently added to aluminum base alloys to improve certain specific properties and also the usual impurities of iron and silicon.

I claim:

1. A magnesium-free aluminum base alloy containing from 1 to 12 per cent copper, from 0.01 to 2 per cent lithium, from 0.01 to 1.5 per cent

cadmium and the balance substantially all aluminum, said alloy being characterized by a higher tensile and yield strength in the heat treated and aged condition than the same alloy not containing both lithium and cadmium.

2. A magnesium-free aluminum base alloy containing from 1 to 12 per cent copper, from 0.01 to 2 per cent lithium, from 0.01 to 0.5 per cent zinc and the balance substantially all aluminum, said alloy being characterized by a higher tensile and yield strength in the heat treated and aged condition than the same alloy not containing both lithium and zinc.

15 3. A magnesium-free aluminum base alloy containing from 1 to 12 per cent copper, from 0.01 to 2 per cent lithium, from 0.02 to 1.5 per cent total of cadmium and zinc, the zinc not exceeding about 0.5 per cent, and the balance substantially all aluminum, said alloy being characterized by a higher tensile and yield strength in the heat treated and aged condition than the same alloy not containing lithium, cadmium and zinc.

20 4. A magnesium-free aluminum base alloy containing from 3 to 5 per cent copper, from 0.01 to 2.0 per cent lithium, at least one of the elements selected from a group consisting of cadmium, mercury, silver, tin, indium and zinc, these elements being present in the proportion of about 0.01 to 1.5 per cent each of cadmium, mercury, silver, tin, indium, and about 0.01 to 0.5 per cent of zinc, the total of these elements not exceeding about 1.5 per cent, and the balance substantially all aluminum, said alloy being characterized by a higher tensile and yield strength in the heat treated and aged condition than the same alloy not containing both lithium and at least one of the metals from said group.

25 5. A magnesium-free aluminum base alloy containing from 3 to 5 per cent copper, from 0.01 to 2 per cent lithium, from 0.01 to 1.5 per cent cadmium and the balance substantially all aluminum, said alloy being characterized by a higher tensile and yield strength in the heat treated and aged condition than the same alloy not containing both lithium and cadmium.

30 45 6. A magnesium-free aluminum base alloy containing from 1 to 12 per cent copper, from 0.01 to 2.0 per cent lithium, at least one of the elements selected from a group consisting of cadmium, mercury, silver, tin, indium and zinc, these elements being present in the proportion of about 0.01 to 1.5 per cent each of cadmium, mercury, silver, tin, indium, and about 0.01 to 0.5 per cent of zinc, the total of these elements not exceeding about 1.5 per cent, and the balance substantially all aluminum, said alloy being characterized by a higher tensile and yield strength in the heat treated and aged condition than the same alloy not containing both lithium and at least one of the metals from said group.

IRA M. LE BARON.